

L. L. SUMMERS.  
PROCESS OF COKING COALS.  
APPLICATION FILED FEB. 18, 1910.

968,499.

Patented Aug. 23, 1910.



WITNESSES:

*Frederick Seegers  
McHugh.*

INVENTOR

*Leland L. Summers  
BY  
Charles J. Fitts.*

ATTORNEY

# UNITED STATES PATENT OFFICE.

LELAND L. SUMMERS, OF CHICAGO, ILLINOIS, ASSIGNOR TO CONTINUOUS PROCESS COKE COMPANY, A CORPORATION OF MAINE.

## PROCESS OF COKING COALS.

968,499.

Specification of Letters Patent. Patented Aug. 23, 1910.

Application filed February 18, 1910. Serial No. 544,625.

To all whom it may concern:

Be it known that I, LELAND L. SUMMERS, a citizen of the United States, residing at Chicago, county of Cook, and State of Illinois, have invented certain new and useful 5 Improvements in the Process of Coking Coals, of which the following is a specification.

The object of my invention is to provide a 10 process of coking by means of which coke may be produced from coals having a comparatively high sulfur or phosphorus content and in particular the object of my invention is to provide a coking process in 15 which the impurities existing in the coals, notably sulfur, phosphorus, iron, and silica, and similar impurities may be removed during the coking process, thus producing coke of suitable character for use as a fuel for 20 metallurgical purposes.

As is well known, sulfur and phosphorus existing in certain coals together with iron, and similar impurities are in such state or combination as to be detrimental to the coking 25 process as carried on in the oven, because owing to the state or combination in which these naturally exist they are not readily volatilized as hereinafter explained.

In general terms, my process consists in 30 providing a method by which such impurities are first acted upon chemically so that their condition is changed and they are removed in part and in part become capable 35 of being volatilized, and then the coals are subjected to the ordinary coking process during which these volatile products are caused to pass off so that they are not precipitated as chemical compounds in the coke.

The general characteristics of phosphorus 40 resemble those of sulfur in forming phosphides and phosphates and also in forming various volatile compounds. Hence, the treatment for the sulfur will ordinarily result in the removal of phosphorus and in 45 this specification the details covering the one will in general apply to the other, particularly as sulfur exists in much greater quantities than phosphorus in coal.

The following explanation in connection 50 with the removal and treatment of sulfur will in general be applicable to the removal and treatment of the phosphorus.

I will describe my invention in connection 55 with an apparatus suitable for the practice of such invention or method, yet it is to be

understood that my invention is not limited in respect to the particular method of partially removing and transforming sulfur and the like into volatile products; nor to any character of apparatus which may be used 60 for this purpose, but that my method may be practiced in other ways.

A portion of the sulfur in the coal ordinarily exists in the form of iron pyrites or bisulfid of iron  $FeS_2$ . Another portion of 65 the sulfur exists as the monosulfid of iron  $FeS$  and still another portion exists as sesquisulfid  $Fe_2S_3$ . The monosulfid is readily decomposed by dilute mineral acids with the evolution of hydrogen sulfid and a salt of 70 the metal, in accordance with the following equations:



75

The monosulfid of iron is not readily oxidized. The bisulfid of iron  $FeS_2$  resists the action of mineral acids, but may be oxidized (in the presence of moisture) to the ferrous 80 sulfate  $FeSO_4$  and the ferric sulfate  $Fe_2(SO_4)_3$ . The sesquisulfid of iron is partially converted into the one and partially into the other form by oxidation and dilute acids. The action of oxygen and water on 85 the bisulfid is expressed by the following equation:



In the carrying out of my improved coking process, I first treat the carbonaceous material to be coked chemically so that reactions similar to those above described may be carried out and the sulfur and phosphorus compounds may be transformed into 90 readily volatilizable substances. I then subject the material so treated to coking temperature in a closed retort during which the said volatilizable substances are driven off and in the coke so formed the deleterious 95 compounds are greatly reduced and coke suitable for use, especially in metallurgical operations, is obtained. I may use any means for effecting the necessary reactions, and will describe one means which may be used.

In the drawings, the figure is a vertical sectional elevation of an apparatus suitable for the practice of my invention.

Referring to the drawings, an electrolytic 110

tank A of any suitable shape and dimensions is provided with revolving electrodes B and C mounted on the shaft D and driven in any desired manner as by the gears E and E' and pulley E<sup>2</sup> which in turn are driven by any suitable source of power (not shown). The electrode B is connected to the positive wire from a suitable source of electrical energy through the contact ring F and brush G and the electrode C is connected with the negative lead from the same source of electrical energy through contact ring F' and brush G'. The electrolytic tank A has a single compartment in which the electrodes of different polarity revolve, but if desired a double compartment may be employed, and the electrodes B and C placed in separate compartments, the products of electrolysis being thus separated, as is well known in the art.

The method so far described is based essentially upon the well known fact that upon the passage of an electric current in a suitable electrolyte, electrolytic decomposition 25 will result.

According to my method as practiced, the coal to be electrolyzed is preferably in a finely subdivided form and is submerged in the electrolyte, so that upon revolving 30 the electrodes B and C a continual agitation of the substance in contact with the products of electrolysis results. The electrolyte used may be varied to suit the substances existing in the coal, and may be conveyed into the tank by any suitable means such as a pump P.

In this method of extracting the sulfur, I preferably use an acid or acid-forming electrolyte such as sulfuric acid in water or 40 any soluble sulfate which will have a combined decomposing action on the sulfids of iron, the acids converting the monosulfid into hydrogen sulfid and a soluble sulfate, at the same time that oxygen and water are decomposing the bisulfid. As the electrolyte is decomposed by the electric current, the acid radical and the oxygen traveling to the positive pole or anode causes an active and effective action on the substances in the 45 vicinity of the anode. Thus, the particles of  $FeS_2$  are oxidized in the electrolyte, the product being soluble ferrous and ferric sulfate and hydrogen sulfid, while the monosulfid of iron is acted upon by the acids. 50 The sulfates, being soluble, are, of course, retained in the electrolytic solution, and are removed with said solution.

The hydrogen sulfid formed by the above reactions is decomposed by the oxygen, in 55 accordance with the following equation:



The result of the action of this electrolyte upon the sulfids of iron has thus been to 60 place the iron in solution and precipitate

the sulfur as free sulfur in a very minute or finely divided state. It is apparent that the coal thus treated when chemically analyzed for sulfur in the ordinary manner would show practically the same sulfur content or but a slightly diminished amount of sulfur over that contained in untreated coal. It is apparent, however, that the sulfur existing in the coal has been changed in its mode of occurrence, so that it no longer is 75 united to iron for which it has a very pronounced chemical affinity or heat of combination. It is also apparent that as the metallic particles have been entirely removed from the coal with which the sulfur will readily combine, the sulfur is free to combine with other substances and upon 80 charging the coal into a coke oven and highly heating the coal, the sulfur may be volatilized and particularly upon intimate 85 contact with large quantities of hydrogen distilled from the coal with which hydrogen, sulfur can readily be caused to unite. The sulfur may, therefore, be distilled from the coal as a volatile compound with hydrogen 90 such as hydrogen sulfid  $H_2S$ , as volatile compound with carbon disulfid  $CS_2$ , or as various hydrocarbon compounds such as thiophen.

In the foregoing description of the electrolytic treatment of the coal I have described one specific chemical treatment for the coal but it is to be understood that I do not intend thereby to limit my process to any special chemical treatment as any suitable method of causing the necessary reactions may be employed.

A suitable oven for heating the carbonaceous material to drive off the volatilizable substances and complete the coking operation is described in my Patent No. 943,610 granted on the 14th day of December, 1909, to which reference is made for a more complete description. This patent shows an apparatus suitable for a continuous coking process in which the carbonaceous material to be coked is fed into the retort and conveyed therethrough while the coking operation is going on. In the drawings, I have illustrated diagrammatically such a coking apparatus, I being the hopper into which the carbonaceous material is conveyed from the electrolytic tank to K, the coking retort. I have not here illustrated the feeding and conveying devices as these are fully shown 110 and described in my patent above referred to.

The carbonaceous material may be conveyed from the electrolytic tank to the hopper by any suitable means. In the drawing, I have illustrated an inclined conveyor floor H down which the material may run from the tank to the hopper. Beneath this conveyor floor I have shown a heating device S, which may be of any suitable construction, such as steam pipes, for the pur- 125 130

pose of drying the material as it passes to the coking apparatus.

The carbonaceous material may be conveyed to the floor H by any suitable means.

5 In the drawing, I have shown the tank as provided with a hinged door W, which may be opened to allow the material in the tank to pass therefrom to the floor H, it being understood, of course, that the solution is 10 drained away, or separated from the material in any suitable manner. As the particular means for accomplishing these results form no part of my present invention, I do not deem it necessary to describe them 15 more fully.

It will be understood that while I have illustrated only one way in which my improved process may be carried out, the process itself is not restricted to the particular form of apparatus herein described 20 and that it may be carried out in widely different forms of apparatus without departing from the spirit of my invention.

I claim:

25 1. The process of coking carbonaceous material containing compounds of sulfur, phosphorus, or the like, which consists in first treating the carbonaceous material to transform the sulfur, phosphorus, or the like 30 in said compounds into volatilizable condition and then subjecting the carbonaceous material to a coking temperature in a closed retort.

2. The process of coking carbonaceous 35 material containing compounds of sulfur, phosphorus, or the like which consists in

first chemically treating the carbonaceous material to transform the sulfur, phosphorus, or the like in said compounds into volatilizable condition, and then heating the 40 said material in a closed retort.

3. The process of coking carbonaceous material, which consists in chemically treating said material to transform its content of sulfur compounds and the like into vola- 45 tilizable condition, then feeding said material to a heated coking retort and conveying the material through said retort.

4. The process of coking carbonaceous material containing compounds of sulfur, 50 phosphorus, or the like, which consists in first treating the carbonaceous material to transform the sulfur, phosphorus, or the like in said compounds into volatilizable condition, drying said material, and then subjecting 55 the carbonaceous material to a coking temperature in a closed retort.

5. The process of coking carbonaceous material containing compounds of sulfur, phosphorus, or the like, which consists in 60 electrolytically treating the carbonaceous material, thereby placing the sulfur, phosphorus, or the like in said compounds in volatilizable condition, and then subjecting the carbonaceous material to a coking tempera- 65 ture in a closed retort whereby the volatilizable substances are driven off.

LELAND L. SUMMERS.

Witnesses:

M. E. STRUTENHUGH,  
W. J. RYAN.